

Patented Dec. 6, 1927.

1,651,990

# UNITED STATES PATENT OFFICE.

PAUL BERTHON, OF LYON, FRANCE, ASSIGNOR TO SOCIÉTÉ DE STEARINERIE & SAVONNERIE DE LYON, OF LYON, FRANCE.

## PROCESS OF MANUFACTURING CELLULOSE ESTERS.

No Drawing. Application filed February 12, 1924, Serial No. 692,440, and in France July 31, 1923.

In my copending applications Serial Nos. 591,426, filed 29 September 1922, and 623,283, filed 6 March 1923, processes for obtaining soluble cellulosic esters from the higher acids 5 and in particular from fatty acids are described.

The present invention has for its object a process of introduction of one or more radicals of the higher fatty acid by esterification 10 not of simple celluloses or carbohydrates as in the above mentioned applications but of celluloses or carbo-hydrates which have been previously esterified either by means of mineral acids, for example nitric acids, or 15 organic acids (other than the higher fatty acids) for example acetic acid, either by means of derivatives of these acids or by any method.

Broadly the invention consists in the 20 esterification of simple or mixed esters of the cellulose  $C_6H_{10}O_5$  modified or not of which the acid radial or radicals may be either mineral acid residues or organic acid residues (other than higher fatty acid residues) by 25 which mixed cellulosic esters of which one residual acid at least is constituted by a higher fatty acid are obtained.

The process is carried out by treating the 30 mineral or organic cellulose esters with fatty acid chlorides in the presence of pyridine and a diluent such for example as benzene, and at a suitable temperature.

The pastry mass obtained at the end of the 35 reaction is then precipitated by alcohol and purified.

The process is essentially different from all those hitherto known and which consisted in causing a mixture of acid chlorides to act simultaneously on cellulose in the presence 40 of pyridine under which conditions it is impossible to determine in advance what will be the exact constitution of the mixed esters which will be formed and in particular the proportion in which the different organic 45 radicals corresponding to the acid chlorides used will be really contained in the ester obtained.

In my process on the contrary the exact 50 composition of the mixed esters prepared can be ascertained in advance; for example by starting with nitro-cellulose containing a

known tenure of the radical  $NO_2$ , the reaction can be effected by introducing a determined proportion of a higher fatty acid radical.

For example starting with nitro or aceto-cellulose containing for each molecule  $C_6H_{10}O_5$  one or two nitric or acetic radicals or both, it is possible to obtain by additional esterification mixed diesters or triesters containing one or two higher fatty acid radicals. 55 60

The mixed esters obtained appear in the shape of fibrous filaments which are formed during the precipitation by the alcohol of the mixed ester in benzene and toluene.

Their solubility is more or less modified 65 but they possess in general the valuable property of being soluble in the aromatic series of hydrocarbons, more particularly benzene.

Their solutions furnish by evaporation 70 transparent and colourless pellicles, the elasticity of which is practically identical and the tenacity greater than that of simple cellulosic esters of the higher fatty acids.

The following is an example of the process:—100 grams of di-nitrocellulose (11.3% 75 about of nitrogen) is dissolved in 200 grams of pyridine and a solution of 300 grams of chloride of lauryl in 300 grams of toluene is added. The mixture is heated for half an hour to one hour to 40–45° C.

The pasty mass thus obtained is recovered 80 by alcohol in the hot state and it is then purified by dissolution in benzene and re-precipitation of the benzene solution by alcohol.

The yield is from 85 to 90%. The lauro-dinitro-cellulose appears in the form of 85 whitish filaments which are sufficiently resistant and the inflammability of which is considerably less than that of nitro-cellulose. Its solubility is the same as that of simple cellulosic esters of the higher fatty acids. 90

What I claim as my invention and desire to secure by Letters Patent of the United States is:—

1. A process for manufacturing mixed cellulose esters soluble in the aromatic series 95 of hydrocarbons, consisting in heating mineral acid cellulose esters together with chlorides of the higher fatty acids in the presence of pyridine and benzene hydrocarbon, precipitating the mass at the end of the reaction 100

by alcohol and purifying the product obtained.

2. Process for manufacturing mixed cellulose esters soluble in the aromatic series of  
5 hydrocarbons, consisting in dissolving di-nitrocellulose in pyridine, adding a solution of chloride of lauryl in toluene, heating the

mixture, precipitating the mass at the end of the reaction by alcohol, purifying the product by dissolution in benzene and precipitating 10 the benzene solution by alcohol.

In witness whereof I have signed this specification.

PAUL BERTHON.